

May 16, 1939.

R. G. BOWMAN ET AL

2,158,269

ELECTROLYTIC PROCESS FOR THE MANUFACTURE OF LITHARGE

Filed Oct. 30, 1935



Anolyte \_\_\_\_\_  
Catholyte \_\_\_\_\_  
Litharge \_\_\_\_\_

INVENTOR  
Reginald G. Bowman  
William J. Knox Jr.  
BY

Pennie, Davis, Mannin & Edmunds  
ATTORNEYS

## UNITED STATES PATENT OFFICE

2,158,269

## ELECTROLYTIC PROCESS FOR THE MANUFACTURE OF LITHARGE

Reginald G. Bowman, Gary, and William J. Knox, Jr., Hammond, Ind., assignors to Anaconda Lead Products Company, New York, N. Y., a corporation of Delaware

Application October 30, 1935, Serial No. 47,340

13 Claims. (Cl. 204—61)

This invention relates to the electrolytic production of litharge, and has for an object the provision of an improved process for producing litharge electrolytically. More particularly, the invention contemplates the provision of a method for the electrolytic production of litharge in accordance with which features of control are provided to insure satisfactory progress of the reactions involved and the efficient production of a final product of uniformly high quality.

For many years commercial litharge has been prepared by direct oxidation of atomized molten lead, or by direct oxidation of a bath of molten lead. The product of these methods does not meet the high standard of purity and uniformity demanded by consumers of litharge, and, as a consequence, manufacturers have had to resort to careful selection and grading of the product, rejecting a considerable portion as unsuited for many of the uses for which high quality litharge is required.

It has been proposed to overcome the disadvantages inherent in the production of litharge by direct oxidation of molten lead by producing litharge electrolytically, but, heretofore, no commercially feasible electrolytic process for the production of litharge has been devised. Probably this has been owing to a lack of understanding of factors influencing the electrolytic reactions occurring during operation of the various processes proposed. Whatever the reason may have been, however, we have found that it is possible so to control the progress of the electrolytic reactions resulting in the production of litharge as to make possible the development of a satisfactory commercial electrolytic process.

Electrolytic litharge is generally produced in a bifluid electrolytic cell, that is, a cell in which two physically separated electrolytes are employed. One of these electrolytes, the anolyte, is in contact with the anode, and the other, the catholyte, is in contact with the cathode. Physical separation of the anolyte and catholyte is effected by means of a permeable or semi-permeable membrane or diaphragm of such nature and so arranged as to permit the passage of electric current from anode to cathode through the anolyte and the catholyte.

The anode comprises a sheet or plate of metallic lead, and the anolyte with which it is in contact comprises an aqueous solution of a salt, for example, an alkali metal salt such as sodium acetate, capable upon electrolysis of providing a solvent for the lead of the anode. The catholyte comprises an aqueous solution of a substance, for

example, sodium hydroxide, capable of acting as a reagent for precipitating the dissolved lead in the anolyte as litharge. The cathode in contact with the catholyte is preferably insoluble in the catholyte and may comprise a thin sheet of copper, iron, or other suitable conducting material.

The diaphragm, which constitutes an important element in bifluid cell construction and operation, advantageously comprises a bag or envelope surrounding one of the electrodes, preferably the cathode. Fabrics such as linen woven to attain an optimum degree of porosity serve admirably for use in the construction of the diaphragm.

The reactions taking place during electrolysis apparently proceed somewhat as follows: When an electric current is passed through a cell of the type described, employing a sodium acetate solution as the anolyte and a solution of sodium hydroxide as the catholyte, lead from the anode dissolves as normal lead acetate, and sodium ions are caused, by the action of the current, to migrate toward the cathode. They pass through the diaphragm and enter the catholyte, wherein, at the cathode, they react with the water present to form sodium hydroxide, liberating hydrogen. The sodium hydroxide thus formed in the catholyte diffuses back through the diaphragm into the anolyte, and there it reacts with the normal lead acetate to form a soluble basic acetate of lead and to regenerate a portion of the sodium acetate. The basic acetate of lead reacts with a further quantity of sodium hydroxide to produce yellow crystalline flakes of litharge, which precipitate from solution, and simultaneously the balance of the sodium acetate is regenerated.

We have found that the above-outlined process will not proceed satisfactorily unless the concentration of dissolved lead in the anolyte is maintained within predetermined limits, and, moreover, satisfactory operation requires that the lead in solution be present as the basic lead ion and not as the plumbite ion. If the anolyte contains an insufficient quantity of basic lead acetate in solution, the rate at which sodium hydroxide migrates from the catholyte into the anolyte is apt to be such that all of the lead will be precipitated, leaving the anolyte alkaline. The lead dissolved at the anode will then be converted to plumbite salts, which are incapable of being precipitated as litharge, and the process will become inoperative. Conversely, if the concentration of basic lead acetate exceeds the maximum allowable limit, local variations in

- temperature and concentration will cause crystallization of the basic lead acetate along with precipitation of litharge, resulting in a contaminated product. Since lead forms a series of basic lead acetates of different solubilities exerting different effects upon the pH of their solutions, it is difficult to define exactly the limits within which the concentration of lead should be maintained. The practical limits between which the concentration of dissolved lead, calculated as metallic lead in the anolyte, should lie, however, have been found to be about 0.1% to 1.0%. Especially satisfactory results have been attained by maintaining the concentration of the dissolved lead at between 0.2% and 0.4%, say about 0.3%, of the weight of the solution.
- In accordance with the present invention, the concentration of dissolved lead in the anolyte is controlled by regulating the rate at which the sodium hydroxide or other litharge precipitant is transferred from the catholyte to the anolyte. This may be accomplished by selecting as the diaphragm a material of suitable porosity, by regulating the extent by which the hydrostatic head of liquid in the catholyte compartment exceeds that of the liquid in the anolyte compartment, by adding catholyte to anolyte at any point outside the reacting zone of the cell, or by employing any suitable combination of these methods of control. Preferably the control afforded by the diaphragm porosity or the hydrostatic head of anolyte with respect to catholyte, or both, should be such that the rate of transfer of hydroxyl ions as effected thereby approximates but does not exceed the rate at which the lead dissolved in the anolyte is capable of combining with said hydroxyl ions to produce litharge. Complete control is then attained by suitable addition of catholyte to anolyte.
- A specific embodiment of the invention is diagrammatically illustrated in the accompanying flowsheet. An electrolytic cell 10 is schematically shown as having a diaphragm 11 to separate an anolyte compartment 12 from a catholyte compartment 13. A lead anode (not shown) is in contact with anolyte within the anolyte compartment 12, and a copper, iron or other suitable insoluble cathode (not shown) is in contact with catholyte within the catholyte compartment 13. (In a commercial cell, of course, there would be a large number of alternate anolyte and catholyte compartments, each compartment containing an anode or a cathode.) The anolyte within the anolyte compartment comprises an aqueous solution containing about ten percent sodium acetate, and the catholyte within the catholyte compartment comprises an aqueous solution containing about five percent sodium hydroxide.
- In order to maintain proper quantities and concentrations of electrolyte within the cell, and to provide for easy recovery of the products of the cell, both anolyte and catholyte are circulated through systems external to the cell itself. A reserve of anolyte is maintained in an anolyte storage tank 14, from which quantities are delivered as required to an anolyte feed tank 15. From the feed tank, anolyte is supplied at a substantially constant rate to the anolyte compartment 12 of the cell. Excess anolyte is permitted to overflow therefrom and run to a settling tank 16, and a further quantity of anolyte, withdrawn either continuously or intermittently from a low point in the anolyte compartment together with the precipitated litharge or other product of the cell, is likewise delivered to the settling tank 16.

Quantities of anolyte may also be passed from the storage tank 14, feed tank 15, or both, directly to the settling tank 16, for reasons explained in detail hereinafter.

In the settling tank 16 the bulk of the litharge or other solid product of the cell settles from the liquid and is withdrawn from a point at or near the bottom of the tank to a filter 17. The supernatant liquor from the settling tank 16, together with such solid material as has not settled, passes to a second settling tank 18. Here the balance of the solid matter settles from the solution and is withdrawn from a point adjacent the bottom of the second settling tank 18 and passed to the filter 17.

The bulk of the liquor still associated with the solid litharge or other product is removed in the filter 17, and the filtered residue is washed with water, preferably countercurrently while still on the filter. The solid product may then be passed to a drying oven 20 to remove the last traces of water, and after drying may be ground if desired in a ball mill 21 or other appropriate grinding apparatus, from which is obtained the final product.

The supernatant liquor from the second settling tank 18 and the anolyte recovered in the filter are united in an anolyte sump 22. Washings from the filter, which contain quantities of the soluble salts of the anolyte, also may advantageously be united with the anolyte in the anolyte sump 22. Anolyte from the sump may be delivered by means of a pump 23 or otherwise to the storage tank 14 for recirculation through the system.

Catholyte is circulated similarly to the anolyte through a system external to the cell. Catholyte from a catholyte storage tank 24 passes to a catholyte feed tank 25 and from there to the catholyte compartment 13 of the cell. Excess catholyte overflows from the catholyte compartment and is delivered to a catholyte sump 26, from which it may be pumped by means of a pump 27 to the catholyte storage tank 24 for recirculation through the system.

A quantity of catholyte is withdrawn from the catholyte feed tank 25 (or from the catholyte storage tank 24 if desired) either continuously or intermittently as may be required and is added to the anolyte withdrawn from the lower portion of the anolyte compartment 12 of the cell. Make-up water is supplied from time to time as needed to the catholyte storage tank 24.

To start the cell in operation, it is necessary to supply dissolved lead in the form of lead acetate to the anolyte. This may be done by simply passing current through the cell to dissolve lead from the anode in the form of lead acetate, while retarding precipitation thereof as litharge until the desired concentration of dissolved lead in the anolyte has been attained. With large volumes of anolyte being circulated, however, considerable time would be required before this could be accomplished, and consequently, it is preferred to make up the anolyte with the proper quantity of lead acetate already dissolved therein. In preparing the anolyte, it has been found best to make up a saturated solution of sodium acetate and to add sufficient lead acetate so that when the solution is diluted to the proper strength for use as the anolyte, the solution will contain about 0.3% of dissolved lead and about 10% sodium acetate, both by weight of the solution. This procedure offers the additional advantages of effecting precipitation as

insoluble lead compounds of any impurities that may be present in the sodium acetate employed (commercial sodium acetate is preferred) such as sulphates, carbonates, and to some extent chlorides, and these precipitated impurities may be separated from the solution before it is introduced into the anolyte circuit.

It is also preferred, especially if the anolyte is prepared as described above, to prepare a concentrated sodium hydroxide solution and to dilute it to the proper strength (about 5% NaOH by weight of the solution) for use as the catholyte. Practically, this procedure is more advantageous than depending upon electrolysis for the production of a suitable catholyte. Sodium carbonate, which is apt to be the principal impurity in the sodium hydroxide employed, may be separated from the concentrated solution prior to dilution for use as the catholyte, in any suitable manner, as by fractional crystallization. After the process has been set in operation, no further addition of reagents (sodium hydroxide and sodium acetate) is necessary.

After the anolyte and catholyte compartments have been filled with anolyte and catholyte, respectively, electrolysis is started by passing an electric current through the cell. Lead dissolves from the anode and litharge commences to form in the anolyte, probably substantially in accordance with the reactions mentioned above. The litharge settles in the anolyte to the lower portion of the cell, from which it is withdrawn together with a quantity of anolyte and is delivered to the first settling tank 16 for purposes of recovery substantially as described above. The recirculating anolyte and catholyte may be used over and over, since the sodium acetate is regenerated and lead acetate and sodium hydroxide are produced by electrolysis in the same chemical proportions as they are consumed in the production of litharge. Thus the only reagents actually consumed are the lead of the anode, which may be replaced by introducing a new anode from time to time as necessary, and water which is decomposed to produce the sodium hydroxide employed in the precipitation of the litharge; water added to the catholyte in the catholyte storage tank or the catholyte feed tank serves to replace the water thus consumed.

As pointed out above, continued successful operation of the cell is dependent upon maintaining the concentration of dissolved lead within proper limits, advantageously about 0.3%. This is accomplished by regulation of the rate at which dissolved lead is removed as litharge from the anolyte with respect to the rate at which it is added to the anolyte by electrolysis. In practice, this means controlling the rate at which hydroxyl ions of the catholyte are transferred to the anolyte. The diaphragm affords an important element of control for this purpose, and it should be selected so as to have about that degree of porosity which will permit migration of sodium hydroxide through it at a rate approximating but not exceeding the rate at which it is required in the anolyte to react with the lead acetate dissolved at the anode. If the diaphragm is sufficiently porous to permit migration of the sodium hydroxide at just the rate at which it is consumed in the anolyte, the entire control of the process hinges upon the diaphragm, and a slight failure thereof may throw the entire process out of balance. If the degree of porosity of the diaphragm exceeds this critical limit, easy control of the process will not be possible. Conse-

quently, it is preferred to employ a diaphragm the porosity of which is slightly less than the critical value, and to make up the deficiency of sodium hydroxide in the anolyte which thereby would otherwise occur by controlling other factors influencing the rate of transfer of sodium hydroxide to the anolyte.

One such factor is the hydrostatic head of the catholyte with respect to the anolyte. It is preferred to maintain the surface of the catholyte in the catholyte compartment at a level slightly higher than level of the surface of anolyte in the anolyte compartment. By properly adjusting the hydrostatic head of the anolyte with respect to the catholyte, a considerable measure of control over the rate of seepage of catholyte to anolyte, and thus of the transfer of hydroxyl ions from catholyte to anolyte, is provided. In general, a hydrostatic head of a few inches in favor of the catholyte will be satisfactory.

In practice it is rather difficult to vary the hydrostatic head of anolyte with respect to catholyte to any very great degree without providing a cell of relatively expensive construction, and furthermore, variations in the hydrostatic head of the catholyte are apt to be sluggish in bringing about the effect they are intended to produce. It is, therefore, preferred to operate the cell in such a manner that, even when the catholyte benefits from a slight hydrostatic head with respect to the anolyte, the rate at which sodium hydroxide migrates through the diaphragm into the catholyte is less than the rate at which it is consumed. Complete balance of the process is then achieved by adding quantities of catholyte containing sodium hydroxide to the anolyte at some point external to the reacting zone of the cell. For this purpose, it is preferred to add catholyte from the catholyte feed tank 25 to the anolyte being discharged from the lower portion of the cell with the litharge formed within the cell. This addition of catholyte to the anolyte is regulated to insure maintaining the concentration of dissolved lead in the anolyte at the optimum value of about 0.3%.

It is also advantageous to deliver anolyte that does not pass through the cell directly to the first settling tank 16, in order that the dissolved lead content thereof may be controlled, and to prevent the accumulation of quantities of anolyte of varying dissolved lead content in the various vessels employed. This method of regulating the dissolved lead concentration in the anolyte is exceedingly flexible and easily carried out, and by employing it a very accurate control of the process may be achieved. If the dissolved lead concentration should decrease unduly, as might occur if an excessive quantity of catholyte were added to the anolyte, it may be allowed to increase slowly by electrolysis, or it may be increased quickly by adding an appropriate amount of acetic acid to the anolyte in the cell.

It is desirable, though not essential, to avoid having to add very large quantities of catholyte to anolyte, for each addition of catholyte increases the bulk of the anolyte and decreases the concentration of sodium acetate therein. This difficulty is not serious, however, because the volume of the anolyte may easily be maintained by permitting evaporation of water therefrom. Furthermore, minor variations in the concentration of sodium acetate in the anolyte do not materially affect the operation of the process.

The concentration of dissolved electrolyte in both anolyte and catholyte is dictated primarily

by economic considerations, balancing ohmic resistance of the electrolyte against losses of electrolyte through spillage. If the concentration of the electrolyte is low, loss through spillage will be low, but the ohmic resistance, and hence the power consumption, will be relatively high. Conversely, a high concentration of electrolyte will result in decreased ohmic resistance and decreased power consumption, but will cause increased loss of electrolyte if substantial spillage occurs. Except for the concentration of dissolved lead in the anolyte, the conditions of operation within rather wide limits are not critical. The process has been found to operate well under the following conditions, but they are presented as an illustration of satisfactory operation and are not to be construed as limiting the invention:

Temperature of electrolytes \_\_\_\_\_ °C 40  
 20 Current density per sq. ft. \_\_\_\_\_ amperes 50  
 Anolyte composition:  
 Sodium acetate \_\_\_\_\_ per cent 10  
 Alkalinity (as NaOH) \_\_\_\_\_ per cent 0.1  
 Catholyte composition, sodium hydroxide  
 25 \_\_\_\_\_ per cent 5

Care should be taken in carrying out the process to avoid the formation of sponge lead at the cathode. This may be accomplished by taking 30 care that anolyte containing dissolved lead does not come in contact with any part of the cell which might act as a cathode. Maintaining a hydrostatic head in the catholyte, thus insuring that seepage through the diaphragm proceeds 35 from catholyte to anolyte and not from anolyte to catholyte, is of value for this reason in addition to the reasons set forth above. It is also advisable to insulate the diaphragm from direct contact with the cathode, and to provide bolts, 40 rods, studs, or other metallic parts which might come in contact with the anolyte with hard rubber or other insulating coverings. To the same end it is advantageous to employ anodes of slightly smaller diameter than the cathodes, thereby to 45 insure that the current will not have to pass around any of the frame parts of the diaphragm, if, as is preferred, the diaphragm is in the form of an envelope surrounding the cathode.

Treatment of the solid product of the cell does 50 not entail particular difficulty. It settles readily from the anolyte, and any standard design of settling tank or thickener may be employed in the recovery thereof. Conical settling tanks have been found to be satisfactory.

The product of the settling tanks filters easily, and any of the commonly available filters may be employed to separate the solid and liquid components thereof; for example, a continuous vacuum filter may be employed successfully. None 55 of the salts present in the anolyte is adsorbed by the solid filtered product, and consequently it may be washed easily and effectively, employing ordinary tap water for the purpose and preferably carrying out the washing step on the countercurrent principle. Substantially all of the 60 sodium acetate may be removed from the solid product by washing and may be returned to the anolyte for reuse. Ordinarily, no precautions need be taken to guard against the presence of 65 carbonate in the wash water, as the quantity of such impurity present in ordinary tap water is so small that it will not cause serious contamination of the litharge. In some localities, however, such precautions may be made necessary by the character of the water available.

Drying of the filtered product may be accomplished in any of the commercially obtainable driers. The only precaution necessary in this operation is to avoid the use of temperatures very greatly in excess of 100° C. A temperature of 5 about 110° C. is very satisfactory, for at this temperature the water is easily driven off and the small quantities of lead hydrate which generally are present are converted to litharge. If the product is heated strongly during the drying 10 thereof, the lead hydrate will be converted to lead peroxide which will contaminate the litharge.

The dried product is normally in a fine state of subdivision, but if it is desired to reduce the size of the particles still further, this may be accomplished by means of suitable grinding equipment, for example a ball mill or a pebble mill. Color changes in the litharge may also be brought about by grinding; for example, yellow litharge 15 can be changed to various shades of buff or 20 salmon.

The process of the invention affords a number of advantages not heretofore attained. The only materials consumed in the process are the lead of the anodes and water. The other reagents are employed cyclically and need not be renewed or replaced except in such quantities as may be lost through spillage. It is not necessary to employ lead of particularly high quality for the anodes, because such impurities as it may 30 contain accumulate as an anode slime which may be removed from the electrolytic cell without contamination of the cell product. It may in some cases be profitable to treat these slimes for the recovery of antimony, bismuth, or other 35 valuable substances which they may contain.

The process proceeds smoothly and may be operated either continuously or intermittently as 40 desired. The rate at which litharge is produced in a given cell may be controlled within limits by regulating the current density and the rate of transfer of sodium hydroxide from anolyte to catholyte, thus permitting some correlation of cell output with the demand for the product at any particular time. The electrolytic efficiency 45 of the process is high and the general operating and labor costs are low; consequently, the process is extremely economical in operation.

The product of the cell is of uniformly high 50 quality. Although yellow crystalline litharge is the preferred cell product in accordance with the present invention, other lead compounds, such, for example, as white lead hydroxide or red litharge, may also be produced by suitably adjusting the concentration of dissolved lead in the anolyte. Physically, the product obtained in accordance with the present invention is very finely 55 divided and of remarkably uniform particle size, well suited to the uses to which litharge ordinarily is put. Chemically the product is extremely pure, being of substantially theoretical 60 chemical composition. It possesses a high degree of solubility in acids, dissolving about ten times faster than ordinary commercial litharge. This property is of considerable value in the preparation of lead salts such as lead nitrate, 65 lead chromate, and the like from litharge. The yellow crystalline litharge produced in accordance with the invention possesses the property of darkening upon exposure to light. The fine yellow crystals of litharge may be converted to the buff color of commercial litharge by grinding, and the shade of color of the final product may be controlled by proper adjustment of the grinding 70 conditions. Consequently, it is possible con- 75

sistently to produce litharge of uniform color characteristics.

We claim:

1. The method of producing litharge which comprises passing an electric current through a cell comprising a lead anode, an anolyte comprising a substance capable of serving upon electrolysis as a solvent for lead, a diaphragm, a catholyte comprising a reagent capable of precipitating litharge, and an insoluble cathode, and controlling the progress of reactions taking place within the cell during electrolysis by maintaining the concentration of dissolved lead in the anolyte between about 0.1% and 1.0%. 5
2. The method of producing litharge which comprises passing an electric current through a cell comprising a lead anode, an anolyte comprising a substance capable of serving upon electrolysis as a solvent for lead, a diaphragm, a catholyte comprising a reagent capable of precipitating litharge, and an insoluble cathode, and controlling the progress of reactions taking place within the cell during electrolysis by maintaining the concentration of dissolved lead in the anolyte between 0.2% and 0.4%. 10
3. The method of producing litharge which comprises passing an electric current through a cell comprising a lead anode, an anolyte comprising a substance capable of serving upon electrolysis as a solvent for lead, a diaphragm, a catholyte comprising a reagent capable of precipitating litharge, and an insoluble cathode, and controlling the progress of reactions taking place within the cell during electrolysis by maintaining the concentration of dissolved lead in the anolyte at about 0.3%. 15
4. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by maintaining a hydrostatic head of catholyte with respect to anolyte in the cell to insure the passage of hydroxyl ions from the catholyte to the anolyte at a rate approximating but not exceeding the rate at which lead dissolved in the anolyte is capable of combining therewith to produce litharge. 20
5. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by maintaining a hydrostatic head of catholyte with respect to anolyte in the cell to insure the passage of hydroxyl ions from the catholyte to the anolyte at a rate approximating but not exceeding a rate sufficient to maintain the concentration of dissolved lead within the anolyte between about 0.1% and 1.0%. 25
6. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by maintaining a hydrostatic head of catholyte with respect to anolyte in the cell to insure the passage of hydroxyl ions from the catholyte to the anolyte at a rate approximating but not exceeding the rate at which lead dissolved in the anolyte is capable of combining therewith to produce litharge, and adding catholyte to the anolyte at a point external to the reacting zones of the cell in amount sufficient to maintain the dissolved lead content of the anolyte within predetermined limits. 30
7. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead within predetermined limits by adding a portion of the catholyte which contains hydroxyl ions to anolyte at a point external to the reacting zones of the cell, said catholyte being added to said anolyte in an amount sufficient to maintain the concentration of dissolved lead in the anolyte between about 0.1% and 1.0%. 35
8. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead within predetermined limits by adding a portion of the catholyte which contains hydroxyl ions to anolyte at a point external to the reacting zones of the cell, said catholyte being added to said anolyte in an amount sufficient to maintain the concentration of dissolved lead in the anolyte between about 0.2% and 0.4%. 40
9. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead within predetermined limits by adding catholyte containing hydroxyl ions to anolyte at a point external to the reacting zones of the cell, said catholyte being added to said anolyte in an amount sufficient to maintain the concentration of dissolved lead in the anolyte at about 0.3%. 45
10. In an electrolytic process for the production of litharge in a bifluid electrolytic cell containing anolyte comprising a substance capable of serving upon electrolysis as a solvent for lead in contact with an anode, catholyte comprising an alkali metal hydroxide in contact with a cathode, and a diaphragm separating the anolyte and catholyte, the improvement which comprises maintaining a hydrostatic head of the catholyte with respect to the anolyte in the cell to insure the passage of hydroxyl ions from the catholyte to the anolyte at a rate approximating but not exceeding the rate at which lead dissolved in the anolyte is capable of combining therewith to produce litharge, and adding catholyte to the anolyte at a point external to the reacting zones of the cell in amount sufficient to maintain the dissolved lead content of the anolyte within predetermined limits. 50
11. In an electrolytic process for the production of litharge in a bifluid electrolytic cell containing anolyte comprising a substance capable upon electrolysis of serving as a solvent for lead in contact with a lead anode, catholyte comprising an alkali metal hydroxide in contact with a cathode, and a diaphragm separating the anolyte and catholyte, the improvement which comprises maintaining a hydrostatic head of the catholyte with respect to the anolyte in the cell 55
12. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by maintaining a hydrostatic head of catholyte with respect to the anolyte in the cell 60
13. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by adding catholyte to the anolyte at a point external to the reacting zones of the cell in amount sufficient to maintain the dissolved lead content of the anolyte within predetermined limits. 65
14. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by adding catholyte to the anolyte at a point external to the reacting zones of the cell in amount sufficient to maintain the dissolved lead content of the anolyte within predetermined limits. 70
15. In an electrolytic process for the production of litharge in a bifluid electrolytic cell comprising an anolyte containing a substance capable upon electrolysis of serving as a solvent for lead and a catholyte containing an alkali metal hydroxide, the improvement which comprises maintaining the concentration of dissolved lead in the anolyte within predetermined limits by adding catholyte to the anolyte at a point external to the reacting zones of the cell in amount sufficient to maintain the dissolved lead content of the anolyte within predetermined limits. 75

- to insure the passage of hydroxyl ions from the catholyte to the anolyte at a rate approximating but not exceeding the rate at which lead dissolved in the anolyte is capable of combining therewith to produce litharge, and adding catholyte to the anolyte at a point external to the reacting zones of the cell in amount sufficient to maintain the dissolved lead content of the anolyte between about 0.1% and 1.0%.
- 10 12. In an electrolytic process for the production of litharge in a bifluid electrolytic cell containing anolyte comprising sodium acetate in contact with a lead anode, catholyte comprising sodium hydroxide in contact with a cathode, and 15 a diaphragm separating the anolyte and catholyte, the improvement which comprises maintaining a hydrostatic head of the catholyte with respect to the anolyte in the cell to insure the passage of hydroxyl ions from the catholyte to

the anolyte at a rate approximating but not exceeding the rate at which lead dissolved in the anolyte is capable of combining therewith to produce litharge, and adding catholyte to the anolyte at a point external to the reacting zones of the cell in amount sufficient to maintain the dissolved lead content of the anolyte between about 0.2% and 0.4%.

13. The method of producing litharge electrolytically which comprises introducing an anolyte 10 containing about 10% sodium acetate into the anolyte compartment of a bifluid electrolytic cell, introducing a catholyte containing about 5% sodium hydroxide into the catholyte compartment of said bifluid electrolytical cell, and establishing a concentration of dissolved lead in the anolyte between 0.2% and 0.4%.

REGINALD G. BOWMAN.  
WILLIAM J. KNOX, JR.